

Sept. 3, 1940.

L. C. ANTRIM

2,213,644

METHOD OF COATING A TRANSFER DEVICE

Filed Dec. 13, 1937

*Fig. 1*



*Fig. 2*



*Fig. 3*



*Fig. 4*



*Fig. 5*



INVENTOR

*Louis C. Antrim,*  
BY *Arthur C. Johnson*  
ATTORNEY

## UNITED STATES PATENT OFFICE

2,213,644

## METHOD OF COATING A TRANSFER DEVICE

Louis C. Antrim, New York, N. Y., assignor to  
 Autographic Register Company, Hoboken, N. J.,  
 a corporation of New Jersey

Application December 13, 1937, Serial No. 179,436

6 Claims. (Cl. 91—68)

This invention relates to manifolding, and more particularly to the method of making transfer devices for use in manifolding.

This application is a continuation-in-part of my copending application Serial No. 740,437, filed August 18, 1934.

The manifolding material per se is disclosed and claimed in divisional application Serial No. 256,956, filed February 17, 1939.

10 In transfer devices, it is desirable that the transfer medium or paper carry a maximum quantity of ink so that the device will last over a considerable period of time. However, it has been found that such transfer paper will produce undesirable smudges and will bleed or lose the ink quite rapidly when in use. To overcome this difficulty, applicant has devised a new transfer sheet and a new method for producing the same.

20 According to the present invention, a porous sheet is impregnated with an oil-soluble ink and is provided with a layer or coating in intimate contact with the sheet providing a porous cover for the sheet which will effectively control the amount of ink permitted to leave the paper when an impression is made from the paper, and which will prevent smudges due to excessive ink on the surfaces of the paper.

The layer or porous cover is composed of finely 30 divided material which is insoluble in the ink solution and which is also incapable of chemical reaction with the constituents of the ink. This material adheres firmly to the paper and is retained thereby for substantially the life of the paper.

The invention also provides a novel method of producing the paper whereby the paper is simultaneously impregnated with the ink solution and coated with the finely divided ink-retarding material. This enables the production of the paper to be effected very rapidly.

According to the method of the present invention, the finely divided material is held in suspension in the ink solution and, as the ink is absorbed in the paper, the finely divided material will be deposited on the surface thereof. It will be seen that the deposit will be in proportion to the amount of ink absorbed in the paper so that, when only a small amount of ink is absorbed, only a thin coating is formed on the surface and, conversely, when a large amount of ink is absorbed, the deposit on the surface will be thicker. The deposit or layer is slightly porous 50 so that it will control the flow of ink from the

paper to another medium when impressions are made therefrom.

If desired, one side of the paper can be rendered nontransferring by providing it with an impervious coating of lacquer or the like, so that, when used in a typewriter, the paper will only make one transfer impression.

Other features and advantages of the invention will be apparent from the specification when considered in connection with the drawing, in which:

Figure 1 is a sheet of paper.

Fig. 2 shows a section of the sheets slightly impregnated with the ink and having a thin coating of insoluble powder on the surface. 15

Fig. 3 shows a section of the paper which is fully impregnated with oil-soluble ink and having a heavy deposit of insoluble powder on the surface.

Fig. 4 shows a section of the paper which has 20 been fully impregnated and coated with the finely divided material and having a backing coat of lacquer thereon.

Fig. 5 shows a view of the paper-inking machine. 25

According to the invention, a paper 10 is used as the base material. The paper is unsized and uncalendered so that it is very porous. It must be understood, however, that any type of porous material may be used, according to this invention.

The paper is usually wound into a roll 11 which is mounted on a spindle 12 at the receiving end of an inking machine 13. A mixture of oil and pigment or dye 14 is mixed and placed in the trough 15. A suitable quantity of finely divided or powdered material, which will not chemically react with the ink solution and which is insoluble in the ink solution, is next mixed with the ink solution in the trough 15 so as to be suspended in the inking solution. The solution and powdered material may be completely mixed before being placed in the trough 15 if desired.

The finely divided material or powder may be a metal such as aluminum or bronze, a metal alloy, a metal oxide such as iron oxide, soap stone, or the like. For example, iron oxide makes a very effective coating material for black transfer paper.

The paper from the roll 11 is passed over a 50 guide roller 16 and into the solution in the trough. A guide roller 17 is mounted so as to be positioned in the trough to hold the material submerged in the mixture. As the paper passes through the mixture, it will absorb the ink and 55

the finely divided material or powder, which is in suspension in the solution, will be deposited on the surface, as shown at 22 in Figs. 2 and 3. Fig. 2 diagrammatically shows the paper in the condition when the ink solution first contacts it and places a light deposit of the powdered material on the surface. Fig. 3 diagrammatically shows the sheet when fully impregnated with the ink and coated with the insoluble powder deposit.

10 As is indicated by these two figures, the amount of powdered material deposited on the surface is in proportion to the amount of ink absorbed by the paper. When a small amount of ink is absorbed by the paper, the light coating 15 of powdered material which is deposited will be sufficient to prevent the paper from smudging or bleeding. However, when a larger amount of ink is absorbed by the paper, to thoroughly saturate the same, the danger of smudging is much 20 greater and a larger amount of coating on the surface is necessary to prevent the smudging or excessive bleeding of the ink. This will be present because the increased absorption of the ink into the paper will be operative to deposit by 25 filtration larger quantities of coating material on the paper, and this will be sufficient to prevent the ink from passing from the paper too freely when used. The amount of ink absorption and coating can be controlled by the speed at which 30 the paper is carried through the solution.

The paper, upon leaving the solution, is passed around a guide roll 18, through a pair of squeezing rollers 19, between a pair of spring-pressed feed rollers 20 and through a pair of felt-covered rollers 21. The paper in leaving the tank has the excess ink squeezed therefrom by the rollers 19, which also function to press the powdered material into more intimate contact with the paper. The layer of finely divided material, when in intimate contact with the paper, will adhere thereto for the life of the paper without the use of adhesives or other bonding means. Should there be any unevenness in the coating or any surplus ink solution on the surface of the 40 strip, it will be absorbed and evenly deposited by the felt rollers 21. The strip is then led to a winding means or other take-up device (not shown) where it is allowed to dry.

This process produces a transfer sheet provided with two transfer sides, each capable of giving an impression. If desired, one surface of the impregnated strip can be rendered nontransferring. This may be done in various ways. For example, a backing material or lacquer 23 can be applied directly to the paper if the backing material or the lacquer is impervious to the ink solution. If the material is not completely impervious to the ink solution or will not properly adhere to the paper, a bonding or filler coat can be first applied to the paper and then the lacquer applied to complete the seal of the back of the paper. This prevents offset impressions when the paper is used in a typewriter or the like.

Variations and modifications may be made 65 within the scope of this invention and portions of the improvements used without others.

I claim:

1. The method of making a transfer device for repeated manifolding use, of the kind including an absorbent paper impregnated with an inking solution, which consists in mixing with the inking solution a quantity of powder of the class including powdered metal, powdered alloy, and powdered metal oxide to cause suspension 70 of said powder in said solution; immersing the

absorbent paper in the mixture of inking solution and powder to cause simultaneous absorption of the inking solution by the paper and precipitation of the powder from the inking solution onto the surface of the paper to form a coating thereon comprised solely of a layer of said powder still pulverous except as wetted by said solution; prolonging the time of such immersion until the desired thickness of wetted pulverous coating is obtained on said surface; and removing the paper from such immersion when the desired thickness of coating is obtained on said surface. 10

2. The method of making a transfer device for repeated manifolding use, of the kind including an absorbent paper impregnated with an inking solution, which consists in mixing with the inking solution a quantity of metallic powder to cause suspension of said powder in said solution; immersing the absorbent paper in the mixture 15 of inking solution and metallic powder to cause simultaneous absorption of the inking solution by the paper and precipitation of the powder from the inking solution onto the surface of a paper to form a coating thereon comprised solely of a layer of said powder still pulverous except as wetted by said solution; prolonging the time of such immersion until the desired thickness of wetted pulverous coating is obtained on said surface; and removing the paper from such immersion 20 when the desired thickness of coating is obtained on said surface. 25

3. In the method of making a transfer device for repeated manifolding use, which device comprises a sheet of absorbent paper impregnated with an inking solution and covered at a transfer surface with a coating of metallic powder still pulverous except as wetted by said solution and acting to partially choke the pores of the paper and regulate the quantity of ink solution 30 given off during a transfer operation, the step of insuring that said coating will correspond in degree of thickness to the degree of absorption of inking solution by the paper; said step consisting of adding said powder to and mixing the 35 same with said inking solution and while said inking solution carries said added powder in suspension therein bringing the paper into absorptive relation to said solution, thereby to insure that as impregnation of the paper with said solution proceeds the powder suspended in the solution will be simultaneously deposited on the paper to form a coating on a surface thereof in such manner that said coating becomes thicker and thicker as more and more of the inking solution 40 is absorbed within the body of the paper. 45

4. The method of making a transfer device for repeated manifolding use, of the kind including an absorbent paper impregnated with an inking solution, which consists in mixing with the inking solution a quantity of powdered alloy to cause suspension of said powder in said solution; immersing the absorbent paper in the mixture of inking solution and powdered alloy to cause simultaneous absorption of the inking solution 50 by the paper and precipitation of the powder from the inking solution onto the surface of the paper to form a coating thereon comprised solely of a layer of said powder still pulverous except as wetted by said solution; prolonging the time of such immersion until the desired thickness of wetted pulverous coating is obtained on said surface; and removing the paper from such immersion when the desired thickness of coating is obtained on said surface. 55

5. The method of making a transfer device for  
repeated manifolding use, of the kind including  
an absorbent paper impregnated with an inking  
solution, which consists in mixing with the inking  
solution a quantity of powdered metal oxide  
5 to cause suspension of said powder in said  
solution; immersing the absorbent paper in the  
mixture of inking solution and powdered metal  
oxide to cause simultaneous absorption of the  
inking solution by the paper and precipitation of  
10 the powder from the inking solution onto the  
surface of the paper to form a coating thereon  
comprised solely of a layer of said powder still  
pulverous except as wetted by said solution; pro-  
15 longing the time of such immersion until the de-  
sired thickness of wetted pulverous coating is  
obtained on said surface; and removing the pa-  
per from such immersion when the desired thick-  
ness of coating is obtained on said surface.
- 20 6. The method of making a transfer device for

repeated manifolding use, of the kind including  
an absorbent paper impregnated with an inking  
solution, which consists in mixing with the inking  
solution a quantity of powdered iron oxide  
to cause suspension of said powder in said solu- 5  
tion; immersing the absorbent paper in the mix-  
ture of inking solution and powdered iron oxide  
to cause simultaneous absorption of the inking  
solution by the paper and precipitation of the  
powder from the inking solution onto the sur- 10  
face of the paper to form a coating thereon  
comprised solely of a layer of said powder still  
pulverous except as wetted by said solution; pro-  
longing the time of such immersion until the de-  
sired thickness of wetted pulverous coating is 15  
obtained on said surface; and removing the paper  
from such immersion when the desired thickness  
of coating is obtained on said surface.

LOUIS C. ANTRIM. 20